



US008257895B2

(12) **United States Patent**  
**Zhou et al.**

(10) **Patent No.:** **US 8,257,895 B2**  
(45) **Date of Patent:** **\*Sep. 4, 2012**

(54) **TONER COMPOSITIONS AND PROCESSES**

(75) Inventors: **Ke Zhou**, Oakville, CA (US); **Edward Graham Zwart**, Mississauga, CA (US); **Karen Ann Moffat**, Brantford, CA (US); **Guerino G. Sacripante**, Oakville, CA (US)

(73) Assignee: **Xerox Corporation**, Norwalk, CT (US)

(\*) Notice: Subject to any disclaimer, the term of this patent is extended or adjusted under 35 U.S.C. 154(b) by 442 days.

This patent is subject to a terminal disclaimer.

(21) Appl. No.: **12/576,289**

(22) Filed: **Oct. 9, 2009**

(65) **Prior Publication Data**

US 2011/0086303 A1 Apr. 14, 2011

(51) **Int. Cl.**

**G03G 9/00** (2006.01)

(52) **U.S. Cl.** ..... **430/110.2**; 430/108.21; 430/109.4; 430/110.1

(58) **Field of Classification Search** ..... 430/108.1, 430/108.21, 108.8, 109.1, 109.4, 110.2

See application file for complete search history.

(56) **References Cited**

U.S. PATENT DOCUMENTS

|             |         |                  |
|-------------|---------|------------------|
| 3,590,000 A | 6/1971  | Palermi et al.   |
| 3,800,588 A | 4/1974  | Larson et al.    |
| 3,847,604 A | 11/1974 | Hagenbach et al. |
| 3,967,962 A | 7/1976  | O'Malley         |
| 4,295,990 A | 10/1981 | Verbeek et al.   |
| 4,298,672 A | 11/1981 | Lu               |
| 4,338,390 A | 7/1982  | Lu               |

|             |         |                            |
|-------------|---------|----------------------------|
| 4,935,326 A | 6/1990  | Creatura et al.            |
| 4,937,166 A | 6/1990  | Creatura et al.            |
| 5,236,629 A | 8/1993  | Mahabadi et al.            |
| 5,260,158 A | 11/1993 | Yamaji et al.              |
| 5,273,853 A | 12/1993 | Urano et al.               |
| 5,278,020 A | 1/1994  | Grushkin et al.            |
| 5,290,654 A | 3/1994  | Sacripante et al.          |
| 5,302,486 A | 4/1994  | Patel et al.               |
| 5,308,734 A | 5/1994  | Sacripante et al.          |
| 5,330,874 A | 7/1994  | Mahabadi et al.            |
| 5,344,738 A | 9/1994  | Kmiecik-Lawrynowicz et al. |
| 5,346,797 A | 9/1994  | Kmiecik-Lawrynowicz et al. |
| 5,348,832 A | 9/1994  | Sacripante et al.          |
| 5,364,729 A | 11/1994 | Kmiecik-Lawrynowicz et al. |
| 5,366,841 A | 11/1994 | Patel et al.               |
| 5,370,963 A | 12/1994 | Patel et al.               |
| 5,403,693 A | 4/1995  | Patel et al.               |

(Continued)

FOREIGN PATENT DOCUMENTS

GB 1442835 7/1976  
(Continued)

OTHER PUBLICATIONS

U.S. Appl. No. 12/718,296, filed Mar. 5, 2010.

(Continued)

*Primary Examiner* — Mark F Huff

*Assistant Examiner* — Stewart Fraser

(74) *Attorney, Agent, or Firm* — Eugene O. Palazzo

(57) **ABSTRACT**

An emulsion aggregation toner composition includes toner particles including: an unsaturated polymeric resin, such as amorphous resins, crystalline resins, and combinations thereof; an optional colorant; an optional wax; an optional coagulant; and an IR absorber. The use of an IR absorber may permit formation of color toners that have uniform gloss and crease properties, i.e., the IR absorbers may prevent gloss and crease differences between color and black toners.

**14 Claims, 2 Drawing Sheets**



## U.S. PATENT DOCUMENTS

|              |         |                            |                  |         |                                 |
|--------------|---------|----------------------------|------------------|---------|---------------------------------|
| 5,405,728 A  | 4/1995  | Hopper et al.              | 6,780,500 B2     | 8/2004  | Dumouchel                       |
| 5,418,108 A  | 5/1995  | Kmiecik-Lawrynowicz et al. | 6,830,860 B2     | 12/2004 | Sacripante et al.               |
| 5,496,676 A  | 3/1996  | Croucher et al.            | 7,029,817 B2     | 4/2006  | Robinson et al.                 |
| 5,501,935 A  | 3/1996  | Patel et al.               | 7,087,354 B2     | 8/2006  | Nakamura et al.                 |
| 5,527,658 A  | 6/1996  | Hopper et al.              | 7,141,761 B1     | 11/2006 | Dirubio et al.                  |
| 5,582,950 A  | 12/1996 | Katagiri et al.            | 7,235,337 B2     | 6/2007  | Kameyama et al.                 |
| 5,585,215 A  | 12/1996 | Ong et al.                 | 7,316,879 B2     | 1/2008  | Nakamura et al.                 |
| 5,607,803 A  | 3/1997  | Murofushi et al.           | 7,329,476 B2     | 2/2008  | Sacripante et al.               |
| 5,650,255 A  | 7/1997  | Ng et al.                  | 7,410,739 B2     | 8/2008  | Makamura et al.                 |
| 5,650,256 A  | 7/1997  | Veregin et al.             | 7,510,811 B2     | 3/2009  | Matsumura et al.                |
| 5,723,253 A  | 3/1998  | Higashino et al.           | 2003/0049553 A1  | 3/2003  | Nakamura et al.                 |
| 5,744,520 A  | 4/1998  | Kmiecik-Lawrynowicz et al. | 2003/0129516 A1  | 7/2003  | Nakamura et al.                 |
| 5,747,215 A  | 5/1998  | Ong et al.                 | 2003/0180645 A1  | 9/2003  | Tavernier et al.                |
| 5,763,133 A  | 6/1998  | Ong et al.                 | 2004/0131962 A1* | 7/2004  | Nakamura et al. .... 430/108.21 |
| 5,766,818 A  | 6/1998  | Smith et al.               | 2004/0142263 A1  | 7/2004  | Mikuriya et al.                 |
| 5,804,349 A  | 9/1998  | Ong et al.                 | 2004/0142266 A1  | 7/2004  | Sacripante et al.               |
| 5,827,633 A  | 10/1998 | Ong et al.                 | 2006/0019187 A1  | 1/2006  | Nakamura                        |
| 5,840,462 A  | 11/1998 | Foucher et al.             | 2006/0204880 A1  | 9/2006  | Mizutani et al.                 |
| 5,853,943 A  | 12/1998 | Cheng et al.               | 2006/0222991 A1  | 10/2006 | Sacripante et al.               |
| 5,853,944 A  | 12/1998 | Foucher et al.             | 2006/0223934 A1  | 10/2006 | Chen et al.                     |
| 5,863,698 A  | 1/1999  | Patel et al.               | 2007/0287089 A1  | 12/2007 | Kimura et al.                   |
| 5,869,215 A  | 2/1999  | Ong et al.                 | 2008/0070142 A1  | 3/2008  | Furuki et al.                   |
| 5,902,710 A  | 5/1999  | Ong et al.                 | 2008/0107989 A1  | 5/2008  | Sacripante et al.               |
| 5,910,387 A  | 6/1999  | Mychaljowskij et al.       | 2008/0107990 A1  | 5/2008  | Field et al.                    |
| 5,916,725 A  | 6/1999  | Patel et al.               | 2008/0199797 A1  | 8/2008  | Sacripante et al.               |
| 5,919,595 A  | 7/1999  | Mychaljowskij et al.       | 2008/0236446 A1  | 10/2008 | Zhou et al.                     |
| 5,922,501 A  | 7/1999  | Cheng et al.               | 2008/0268365 A1  | 10/2008 | Yamazaki et al.                 |
| 5,925,488 A  | 7/1999  | Patel et al.               | 2009/0186289 A1* | 7/2009  | Nakamura et al. .... 430/108.4  |
| 5,928,829 A  | 7/1999  | Cheng et al.               | 2009/0220882 A1  | 9/2009  | Zhou et al.                     |
| 5,977,210 A  | 11/1999 | Patel et al.               | 2009/0246679 A1* | 10/2009 | Nosella et al. .... 430/137.14  |
| 6,063,827 A  | 5/2000  | Sacripante et al.          | 2009/0305159 A1  | 12/2009 | Zhou et al.                     |
| 6,214,507 B1 | 4/2001  | Sokol et al.               | 2010/0055593 A1* | 3/2010  | Zhou et al. .... 430/108.4      |
| 6,576,389 B2 | 6/2003  | Vanbesien et al.           | 2011/0086302 A1* | 4/2011  | Zhou et al. .... 430/105        |
| 6,593,049 B1 | 7/2003  | Veregin et al.             | 2011/0086303 A1  | 4/2011  | Zhou et al.                     |
| 6,617,092 B1 | 9/2003  | Patel et al.               |                  |         |                                 |
| 6,627,373 B1 | 9/2003  | Patel et al.               |                  |         |                                 |
| 6,638,677 B2 | 10/2003 | Patel et al.               |                  |         |                                 |
| 6,656,657 B2 | 12/2003 | Patel et al.               |                  |         |                                 |
| 6,656,658 B2 | 12/2003 | Patel et al.               |                  |         |                                 |
| 6,664,017 B1 | 12/2003 | Patel et al.               |                  |         |                                 |
| 6,673,505 B2 | 1/2004  | Jiang et al.               |                  |         |                                 |
| 6,704,538 B2 | 3/2004  | Nakamura et al.            |                  |         |                                 |
| 6,730,450 B1 | 5/2004  | Moffat et al.              |                  |         |                                 |
| 6,743,559 B2 | 6/2004  | Combes et al.              |                  |         |                                 |
| 6,756,176 B2 | 6/2004  | Stegamat et al.            |                  |         |                                 |

## FOREIGN PATENT DOCUMENTS

|    |               |         |
|----|---------------|---------|
| JP | 05-100487     | 4/1993  |
| JP | 06-222616 A   | 8/1994  |
| JP | 06-250547 A   | 9/1994  |
| JP | 2009-251138 A | 10/2009 |

## OTHER PUBLICATIONS

Office Action mailed May 18, 2011 in U.S. Appl. No. 12/718,296. Dec. 14, 2011 Office Action issued in U.S. Appl. No. 12/718,296.

\* cited by examiner

**FIG. 1****FIG. 2**



**FIG. 3**

## 1

## TONER COMPOSITIONS AND PROCESSES

## BACKGROUND

This disclosure is generally directed to toner processes, and more specifically, emulsion aggregation and coalescence processes, as well as toner compositions formed by such processes and development processes using such toners.

Emulsion aggregation/coalescing processes for the preparation of toners are illustrated in a number of Xerox patents, such as U.S. Pat. Nos. 5,290,654, 5,278,020, 5,308,734, 5,370,963, 5,344,738, 5,403,693, 5,418,108, 5,364,729, and 5,346,797; and also of interest may be U.S. Pat. Nos. 5,348,832; 5,405,728; 5,366,841; 5,496,676; 5,527,658; 5,585,215; 5,650,255; 5,650,256 5,501,935; 5,723,253; 5,744,520; 5,763,133; 5,766,818; 5,747,215; 5,827,633; 5,853,944; 5,804,349; 5,840,462; 5,869,215; 5,863,698; 5,902,710; 5,910,387; 5,916,725; 5,919,595; 5,925,488 and 5,977,210. Other patents disclosing exemplary emulsion aggregation/coalescing processes include, for example, U.S. Pat. Nos. 6,730,450, 6,743,559, 6,756,176, 6,780,500, 6,830,860, and 7,029,817.

The disclosures of each of the foregoing patents and publications are hereby incorporated by reference herein in their entireties. The appropriate components and process aspects of the each of the foregoing patents and publications may also be selected for the present compositions and processes in embodiments thereof.

In a number of electrophotographic engines and processes, toner images may be applied to substrates. The toners may then be fused to the substrate by heating the toner with a contact fuser or a non-contact fuser, wherein the transferred heat melts the toner mixture onto the substrate. Electrophotographic digital printing with current toners can produce a range of print gloss when fused using contact fusers such as rolls or belt based fusing sub-systems. The desired gloss level depends on specific customer applications.

To date, toners that are fused with non-contact fusing sub-systems such as flash fusing, radiant fusing or steam fusing sub-systems produce prints that are matte or require very long (2 second) dwell times. Moreover, non-contact fusing systems sometimes utilize high speed continuous feed systems. At high print speeds, colored toners (cyan (C), magenta (M) and yellow (Y)) have lower light-absorbing capacity than a black toner (carbon black absorbs energy), and thus fail to absorb sufficient light to convert energy into heat, resulting in insufficient melting or fixing in the fusing step. A gloss difference between color toners and black toners may also occur due to different light-absorbing capacities of different pigments.

Simply increasing emission intensity of a photo-fixer may generate excessive heat from a black toner as a result of absorbing an excessive quantity of light, causing printing defects referred to as voids or toner bursts on the image. When emission intensity during the fusing step is lowered to an extent to avoid formation of voids by the black toner, insufficient melting or resin flow of the color toners, especially magenta and yellow toners, may be observed. This is because the magenta and yellow toners, which have lower visible light absorbing capacity than a black or cyan toner, cannot absorb sufficient light to melt or cause resin flow.

Toners that are fixed to paper with non-contact fusing having high print gloss with short dwell times remain desirable.

## SUMMARY

The present disclosure provides toners and a printing apparatus utilizing such toners. In embodiments, a toner of the

## 2

present disclosure may include at least one amorphous resin; at least one infrared absorber; at least one crystalline resin; an optional colorant; and an optional wax, wherein the at least one infrared absorber has a maximum absorption of light at wavelengths of from about 700 nm to about 850 nm.

In other embodiments, a toner of the present disclosure may include at least one amorphous polyester resin; at least one infrared absorber; at least one crystalline polyester resin; an optional colorant; and an optional wax, wherein the at least one infrared absorber has a maximum absorption of light at wavelengths of from about 700 nm to about 850 nm and does not absorb light at wavelengths of from about 380 nm to about 700 nm.

A printing apparatus of the present disclosure may include at least one heating device; a toner source; an optional contact fuser; a non-contact fuser comprising a source of infrared light operating at a wavelength of from about 750 nm to about 2500 nm; a substrate pre-heater; an image bearing member pre-heater; and a transfuser, wherein the toner includes at least one amorphous polyester resin, at least one infrared absorber, at least one crystalline polyester resin, an optional colorant and an optional wax, and wherein the at least one infrared absorber has a maximum absorption of light at wavelengths of from about 700 nm to about 850 nm and does not absorb light at wavelengths of from about 380 nm to about 700 nm.

## BRIEF DESCRIPTION OF THE DRAWINGS

Various embodiments of the present disclosure will be described herein below with reference to the figures wherein:

FIG. 1 is a graph of a UV-vis-NIR spectrum of an infrared (IR) absorber which may be utilized in accordance with the present disclosure;

FIG. 2 is a graph of a UV-vis-NIR spectrum of an amorphous resin without a pigment or infrared (IR) absorber; and

FIG. 3 is a graph of a UV-vis-NIR spectrum of a resin of the present disclosure including an amorphous resin and an infrared (IR) absorber.

## DETAILED DESCRIPTION

The present disclosure provides a toner design for non-contact fusing that produces high print gloss in short dwell times. To date, toners that are fused with non-contact fusing sub-systems such as flash/radiant fusing produce prints that are matte or require very long (2 second) dwell times. In accordance with the present disclosure, energy absorbing materials may be included in conventional colored toners to meet the non-contact fusing requirements. In embodiments, to prevent gloss and crease differences between color and black toners, infrared (IR) absorbers are added to color toner(s).

In embodiments the present disclosure is directed to curable toner compositions, including those made by a chemical process such as emulsion aggregation, wherein the resultant toner composition includes an unsaturated polyester resin, an IR absorber, optionally a wax, and optionally a colorant.

Processes of the present disclosure may include aggregating particles, in embodiments particles containing an unsaturated resin such as an unsaturated crystalline or amorphous polymeric resin, in embodiments polyesters, an IR absorber, optionally a wax, and optionally a colorant, in the presence of a coagulant.

A number of advantages may be associated with the toner obtained by the processes and toner compositions illustrated herein. The process allows for particles to be prepared in the

size of from about 2.5 to about 9 microns in diameter, in embodiments from about 3 to about 6 microns in diameter, with narrow size distributions, such as from about 1.2 to about 1.25, without the use of classifiers. Furthermore, low melting or ultra-low melting fixing temperatures can be obtained by the use of crystalline resins in the toner composition. The aforementioned low fixing temperatures allow for non-contact fusing. The toner compositions provide other advantages, such as high temperature document offset properties, in embodiments up to about 85° C., as well as resistance to organic solvents such as methyl ethyl ketone (MEK).

In embodiments, toners prepared in accordance with the present disclosure may be low melt EA toners including an unsaturated resin, an IR absorber, and a shell.

#### Resin

Toners of the present disclosure may include any resin suitable for use in forming a toner. Such resins, in turn, may be made of any suitable monomer. Suitable monomers useful in forming the resin include, but are not limited to, acrylonitriles, diols, diacids, diamines, diesters, diisocyanates, combinations thereof, and the like. Any monomer employed may be selected depending upon the particular polymer to be utilized.

In embodiments, the polymer utilized to form the resin may be a polyester resin. Suitable polyester resins include, for example, sulfonated, non-sulfonated, crystalline, amorphous, combinations thereof, and the like. The polyester resins may be linear, branched, combinations thereof, and the like. Polyester resins may include, in embodiments, those resins described in U.S. Pat. Nos. 6,593,049 and 6,756,176, the disclosures of each of which are hereby incorporated by reference in their entirety. Suitable resins may also include a mixture of an amorphous polyester resin and a crystalline polyester resin as described in U.S. Pat. No. 6,830,860, the disclosure of which is hereby incorporated by reference in its entirety.

In embodiments, the resin may be a polyester resin formed by reacting a diol with a diacid or diester in the presence of an optional catalyst. For forming a crystalline polyester, suitable organic diols include aliphatic diols having from about 2 to about 36 carbon atoms, such as 1,2-ethanediol, 1,3-propanediol, 1,4-butanediol, 1,5-pentanediol, 1,6-hexanediol, 1,7-heptanediol, 1,8-octanediol, 1,9-nanediol, 1,10-decanediol, 1,12-dodecanediol, ethylene glycol, combinations thereof, and the like. The aliphatic diol may be, for example, selected in an amount of from about 40 to about 60 mole percent, in embodiments from about 42 to about 55 mole percent, in embodiments from about 45 to about 53 mole percent of the resin.

Examples of organic diacids or diesters selected for the preparation of the crystalline resins include oxalic acid, succinic acid, glutaric acid, adipic acid, suberic acid, azelaic acid, fumaric acid, maleic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid may be present, for example, in an amount of, for example, in embodiments from about 40 to about 60 mole percent, in embodiments from about 42 to about 55 mole percent, in embodiments from about 45 to about 53 mole percent.

Examples of crystalline resins include polyesters, polyamides, polyimides, polyolefins, polyethylene, polybutylene, polyisobutylene, ethylene-propylene copolymers, ethylene-vinyl acetate copolymers, polypropylene, mixtures thereof, and the like. Specific crystalline resins may be polyester

based, such as poly(ethylene-adipate), poly(propylene-adipate), poly(butylene-adipate), poly(pentylene-adipate), poly(hexylene-adipate), poly(octylene-adipate), poly(ethylene-succinate), polypropylene-succinate), poly(butylene-succinate), poly(pentylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfoisophthaloyl)-copoly(ethylene-adipate), poly(decylene-sebacate), poly(decylene-decanoate), poly(ethylene-decanoate), poly(ethylene-dodecanoate), poly(nonylene-sebacate), poly(nonylene-decanoate), copoly(ethylene-fumarate)-copoly(ethylene-sebacate), copoly(ethylene-fumarate)-copoly(ethylene-decanoate), copoly(ethylene-fumarate)-copoly(ethylene-dodecanoate), and combinations thereof. The crystalline resin may be present, for example, in an amount of from about 5 to about 50 percent by weight of the toner components, in embodiments from about 10 to about 35 percent by weight of the toner components. The crystalline resin can possess various melting points of, for example, from about 30° C. to about 120° C., in embodiments from about 50° C. to about 90° C. The crystalline resin may have a number average molecular weight (Mn), as measured by gel permeation chromatography (GPC) of, for example, from about 1,000 to about 50,000, in embodiments from about 2,000 to about 25,000, and a weight average molecular weight (Mw) of, for example, from about 2,000 to about 100,000, in embodiments from about 3,000 to about 80,000, as determined by Gel Permeation Chromatography using polystyrene standards. The molecular weight distribution (Mw/Mn) of the crystalline resin may be, for example, from about 2 to about 6, in embodiments from about 3 to about 4.

Examples of diacid or diesters selected for the preparation of amorphous polyesters include dicarboxylic acids or diesters such as terephthalic acid, phthalic acid, isophthalic acid, fumaric acid, maleic acid, succinic acid, itaconic acid, succinic acid, succinic anhydride, dodecylsuccinic acid, dodecylsuccinic anhydride, glutaric acid, glutaric anhydride, adipic acid, pimelic acid, suberic acid, azelaic acid, dodecanediacid, dimethyl terephthalate, diethyl terephthalate, dimethylisophthalate, diethylisophthalate, dimethylphthalate, phthalic anhydride, diethylphthalate, dimethylsuccinate, dimethylfumarate, dimethylmaleate, dimethylglutarate, dimethyladipate, dimethyl dodecylsuccinate, and combinations thereof. The organic diacid or diester may be present, for example, in an amount from about 40 to about 60 mole percent of the resin, in embodiments from about 42 to about 55 mole percent of the resin, in embodiments from about 45 to about 53 mole percent of the resin.

Examples of diols utilized in generating the amorphous polyester include 1,2-propanediol, 1,3-propanediol, 1,2-butanediol, 1,3-butanediol, 1,4-butanediol, pentanediol, hexanediol, 2,2-dimethylpropanediol, 2,2,3-trimethylhexanediol, heptanediol, dodecanediol, bis(hydroxyethyl)-bisphenol A, bis(2-hydroxypropyl)-bisphenol A, 1,4-cyclohexanediethanol, 1,3-cyclohexanediethanol, xylenedimethanol, cyclohexanediol, diethylene glycol, bis(2-hydroxyethyl) oxide, dipropylene glycol, dibutylene, and combinations thereof. The amount of organic diol selected can vary, and may be present, for example, in an amount from about 40 to about 60 mole percent of the resin, in embodiments from about 42 to about 55 mole percent of the resin, in embodiments from about 45 to about 53 mole percent of the resin.

Polycondensation catalysts which may be utilized for either the crystalline or amorphous polyesters include tet-

raalkyl titanates, dialkyltin oxides such as dibutyltin oxide, tetraalkyltins such as dibutyltin dilaurate, and dialkyltin oxide hydroxides such as butyltin oxide hydroxide, aluminum alkoxides, alkyl zinc, dialkyl zinc, zinc oxide, stannous oxide, or combinations thereof. Such catalysts may be utilized in amounts of, for example, from about 0.01 mole percent to about 5 mole percent based on the starting diacid or diester used to generate the polyester resin.

In embodiments, suitable amorphous resins include polyesters, polyamides, polyimides, polyolefins, polyethylene, polybutylene, polyisobutylene, ethylenepropylene copolymers, ethylene-vinyl acetate copolymers, polypropylene, combinations thereof, and the like.

In embodiments, an unsaturated, amorphous polyester resin may be utilized as a resin. Examples of such resins include those disclosed in U.S. Pat. No. 6,063,827, the disclosure of which is hereby incorporated by reference in its entirety. Exemplary unsaturated amorphous polyester resins include, but are not limited to, poly(propoxylated bisphenol co-fumarate), poly(ethoxylated bisphenol co-fumarate), poly(butyloxylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butyloxylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butyloxylated bisphenol co-itaconate), poly(co-propoxylated bisphenol co-ethoxylated bisphenol co-itaconate), poly(1,2-propylene itaconate), and combinations thereof. In embodiments, the amorphous resin utilized in the core may be linear.

In embodiments, a suitable amorphous polyester resin may be a poly(propoxylated bisphenol A co-fumarate) resin having the following formula (I):



wherein m may be from about 5 to about 1000, although m can be outside of this range. Examples of such resins and processes for their production include those disclosed in U.S. Pat. No. 6,063,827, the disclosure of which is hereby incorporated by reference in its entirety.

An example of a linear propoxylated bisphenol A fumarate resin which may be utilized as a resin is available under the trade name SPARII from Resana S/A Industrias Quimicas, Sao Paulo Brazil. Other propoxylated bisphenol A fumarate resins that may be utilized and are commercially available include GTUF and FPESL-2 from Kao Corporation, Japan, and XP777 from Reichhold, Research Triangle Park, N.C. and the like.

In embodiments, a suitable amorphous resin utilized in a toner of the present disclosure may have a weight average molecular weight of from about 10,000 to about 100,000, in embodiments from about 15,000 to about 30,000.

Suitable crystalline resins include those disclosed in U.S. Patent Application Publication No. 2006/0222991, the disclosure of which is hereby incorporated by reference in its

entirety. In embodiments, a suitable crystalline resin may be composed of ethylene glycol and a mixture of dodecanedioic acid and fumaric acid co-monomers with the following formula:



wherein b is from about 5 to about 2000 and d is from about 5 to about 2000.

In embodiments, a suitable crystalline resin utilized in a toner of the present disclosure may have a weight average molecular weight of from about 10,000 to about 100,000, in embodiments from about 15,000 to about 30,000.

One, two, or more resins may be used in forming a toner. In embodiments where two or more resins are used, the resins may be in any suitable ratio (e.g., weight ratio) such as, for instance, from about 1% (first resin)/99% (second resin) to about 99% (first resin)/1% (second resin), in embodiments from about 10% (first resin)/90% (second resin) to about 90% (first resin)/10% (second resin).

In embodiments, a suitable toner of the present disclosure may include 2 amorphous polyester resins and a crystalline polyester resin. The weight ratio of the three resins may be from about 29% first amorphous resin/69% second amorphous resin/2% crystalline resin, to about 60% first amorphous resin/20% second amorphous resin/20% crystalline resin, in embodiments from about 45% first amorphous resin/45% second amorphous resin/10% crystalline resin, to about 40% first amorphous resin/40% second amorphous resin/20% crystalline resin.



As noted above, in embodiments, the resin may be formed by emulsion aggregation methods. Utilizing such methods, the resin may be present in a resin emulsion, which may then be combined with other components and additives to form a toner of the present disclosure.

The polymer resin may be present in an amount of from about 65 to about 95 percent by weight, or preferably from about 75 to about 85 percent by weight of the toner particles (that is, toner particles exclusive of external additives) on a solids basis. The ratio of crystalline resin to amorphous resin can be in the range from about 1:99 to about 30:70, such as from about 5:95 to about 25:75.

It has also been found that a polymer with a low acid number may provide better crosslinking results under irradiation. For example, the acid number of the polymer may be from about 0 to about 40 mg KOH/gram, in embodiments from about 1 to about 30 mg KOH/gram, in embodiments from about 5 to about 25 mg KOH/gram, in other embodiments about 7 to about 14 mg KOH/gram.

## IR Absorbers

In accordance with the present disclosure, at least one infrared (IR) absorber is added to a toner for non-contact fusing. An IR absorber may be added to at least one colored toner, in embodiments multiple colored toners. Varying the loading of IR absorber in each colored toner should allow the particles to heat more uniformly amongst the different colored toners, and may heat clear particles more efficiently as well.

The boundaries of the visible region of the absorption spectrum are from about 380 nm to about 700 nm, which correspond to energy boundaries of from about 3.26 eV to about 1.77 eV. For organic molecules, the major contribution to the longest wavelength electronic transition is the transition from HOMO (highest occupied molecular orbital) to LUMO (lowest unoccupied molecular orbital). Therefore, for UV absorbers (absorption<380 nm), the HOMO-LUMO transition energy is greater than about 3.26 eV; for a visible dye or pigment, the HOMO-LUMO transition energy (or band gap) is from about 3.26 eV to about 1.77 eV; for an IR absorber, the HOMO-LUMO transition should be less than about 1.77 eV. In order to reduce the HOMO-LUMO transition energy, a powerful electron donating group containing a "p" lone pair of electrons may be introduced to form a delocalized pi-conjugated system. However, this increased conjugation also reduces the energy difference between the other molecular orbitals, such as the HOMO-Near LUMO (NLUMO) transition energy. When HOMO-LUMO transition energy is slightly less than about 1.77 eV, which may be found for IR absorbers with absorption from about 800 to about 850 nm, the HOMO-NLUMO transition energy could be still larger than about 3.26 eV. However, when the HOMO-LUMO transition energy is less than about 1.77 eV, the HOMO-NLUMO transition energy is less than about 3.26 eV. In those instances, the transition energy occurs in the visible region of the spectrum, giving rise to color. Therefore, in embodiments, an IR absorber with an absorption maximum around 800 nm may be utilized to ensure there is no addition of color in the visible region.

In embodiments, the IR absorber utilized in a toner of the present disclosure may have a maximum absorption at wave-

lengths from about 700 nm to about 850 nm, in embodiments from about 725 nm to about 825 nm, in embodiments from about 730 nm to about 800 nm. In embodiments, the IR absorber utilized in a toner of the present disclosure has no absorption in the visible region of light, i.e., at a wavelength from about 380 nm to about 700 nm.

Suitable IR absorbers having a maximum absorption around 800 nm that may be used include, for example, cyanines, platinum containing dyes, combinations thereof, and the like. Examples of commercially available IR absorbers having a maximum absorption peak at about 800 nm and little absorbing in the visible region of light, i.e., from about 380 nm to about 700 nm, include EPOLIGHT™ 5588 and platinum containing dyes such as EPOLIGHT™ 4113 from EPOLIN, Inc.; SDA9393, SDA6533, SDA1217, SDA2441, SDA7847, SDA1816, SDA4301, SDA4639, SDA2046, SDA5688, SDA8700, SDA8435, and SDA3535 from H.W. Sands; 2-[2-[2-chloro-3-[2-(1,3-dihydro-3,3-dimethyl-1-ethyl-2H-benz[e]indol-2-ylidene)ethylidene]-1-cyclohexen-1-yl]-ethenyl]-3,3-dimethyl-1-ethyl-benz[e]indolium iodide (commercially available as ADS815EI from American Dye Source, Inc.); and cyanines such as NK-2911 and NK-4680 from Hayashibara Biochemical Laboratories, Inc. For reference, the chemical structure of ADS815EI from American Dye Source, Inc. is as follows:



the chemical structure of NK-2911 from Hayashibara Biochemical Laboratories is as follows:



and the chemical structure of NK-4680 from Hayashibara Biochemical Laboratories is as follows:



4% by weight of the toner composition, in embodiments from about 1% to about 3% by weight of the toner composition.

The amount of IR absorber utilized may depend upon the toner to which it is added. In embodiments, the IR absorber may be added so that it is present in an amount of from about 0.01 percent by weight to about 5 percent by weight of the toner, in embodiments from about 0.10 percent by weight to about 1 percent by weight of the toner, in embodiments from about 0.2 percent by weight to about 0.3 percent by weight of the toner. Different colors may have different levels of IR absorbers. Thus, a cyan toner may have an IR absorber in an amount from from about 0.01 percent by weight to about 5 percent by weight of the toner, in embodiments from about 0.10 percent by weight to about 2 percent by weight of the toner, in embodiments from about 0.2 percent by weight to about 0.5 percent by weight of the toner, a magenta toner may have an IR absorber in an amount from about 0.01 percent by weight to about 2 percent by weight of the toner, in embodiments from about 0.10 percent by weight to about 1 percent by weight of the toner, in embodiments from about 0.2 percent by weight to about 0.5 percent by weight of the toner; and a yellow toner may have an IR absorber in an amount from from about 0.01 percent by weight to about 2 percent by weight of the toner, in embodiments from about 0.10 percent by weight to about 1 percent by weight of the toner, in embodiments from about 0.2 percent by weight to about 0.5 percent by weight of the toner;

#### Toner

The resin of the resin emulsions described above, in embodiments a polyester resin, may be utilized to form toner compositions. Such toner compositions may include optional colorants, waxes, and other additives. Toners may be formed utilizing any method within the purview of those skilled in the art including, but not limited to, emulsion aggregation methods.

#### Surfactants

In embodiments, colorants, waxes, and other additives utilized to form toner compositions may be in dispersions including surfactants. Moreover, toner particles may be formed by emulsion aggregation methods where the resin and other components of the toner, including at least one IR absorber, are placed in one or more surfactants, an emulsion is formed, toner particles are aggregated, coalesced, optionally washed and dried, and recovered.

One, two, or more surfactants may be utilized. The surfactants may be selected from ionic surfactants and nonionic surfactants. Anionic surfactants and cationic surfactants are encompassed by the term "ionic surfactants." In embodiments, the surfactant may be utilized so that it is present in an amount of from about 0.01% to about 5% by weight of the toner composition, for example from about 0.75% to about

Examples of nonionic surfactants that can be utilized include, for example, polyacrylic acid, methalose, methyl cellulose, ethyl cellulose, propyl cellulose, hydroxy ethyl cellulose, carboxy methyl cellulose, polyoxyethylene cetyl ether, polyoxyethylene lauryl ether, polyoxyethylene octyl ether, polyoxyethylene octylphenyl ether, polyoxyethylene oleyl ether, polyoxyethylene sorbitan monolaurate, polyoxyethylene stearyl ether, polyoxyethylene nonylphenyl ether, dialkylphenoxy poly(ethyleneoxy) ethanol, available from Rhone-Poulenc as IGEPAL CA210<sup>TM</sup>, IGEPAL CA520<sup>TM</sup>, IGEPAL CA-720<sup>TM</sup>, IGEPAL CO890<sup>TM</sup>, IGEPAL CO720<sup>TM</sup>, IGEPAL CO290<sup>TM</sup>, IGEPAL CA210<sup>TM</sup>, ANTAROX890<sup>TM</sup> and ANTAROX 897<sup>TM</sup>. Other examples of suitable nonionic surfactants include a block copolymer of polyethylene oxide and polypropylene oxide, including those commercially available as SYNPERONIC PE/F, in embodiments SYNPERONIC PE/F 108.

Anionic surfactants which may be utilized include sulfates and sulfonates, sodium dodecylsulfate (SDS), sodium dodecylbenzene sulfonate, sodium dodecylnaphthalene sulfate, dialkyl benzenealkyl sulfates and sulfonates, acids such as abitic acid available from Aldrich, NEOGEN R<sup>TM</sup>, NEOGEN SCT<sup>TM</sup> obtained from Daiichi Kogyo Seiyaku, combinations thereof, and the like. Other suitable anionic surfactants include, in embodiments, DOWFAX<sup>TM</sup> 2A1, an alkylidiphenyloxide disulfonate from The Dow Chemical Company, and/or TAYCA POWER BN2060 from Tayca Corporation (Japan), which are branched sodium dodecyl benzene sulfonates. Combinations of these surfactants and any of the foregoing anionic surfactants may be utilized in embodiments.

Examples of the cationic surfactants, which are usually positively charged, include, for example, alkylbenzyl dimethyl ammonium chloride, dialkyl benzenealkyl ammonium chloride, lauryl trimethyl ammonium chloride, alkylbenzyl methyl ammonium chloride, alkyl benzyl dimethyl ammonium bromide, benzalkonium chloride, cetyl pyridinium bromide, C<sub>12</sub>, C<sub>15</sub>, C<sub>17</sub> trimethyl ammonium bromides, halide salts of quaternized polyoxyethylalkylamines, dodecylbenzyl triethyl ammonium chloride, MIRAPOL<sup>TM</sup> and ALKAQUAT<sup>TM</sup>, available from Alkaril Chemical Company, SANIZOL<sup>TM</sup> (benzalkonium chloride), available from Kao Chemicals, and the like, and mixtures thereof.

#### Colorants

As the colorant to be added, various known suitable colorants, such as dyes, pigments, mixtures of dyes, mixtures of pigments, mixtures of dyes and pigments, and the like, may be included in the toner. The colorant may be included in the toner in an amount of, for example, about 0.1 to about 35

## 11

percent by weight of the toner, or from about 1 to about 15 weight percent of the toner, or from about 3 to about 10 percent by weight of the toner.

As examples of suitable colorants, mention may be made of carbon black like REGAL 330®; magnetites, such as Mobay magnetites MO8029™, MO8060™; Columbian magnetites; MAPICO BLACK™ and surface treated magnetites; Pfizer magnetites CB4799™, CB5300™, CB5600™, MCX6369™; Bayer magnetites, BAYFERROX8600™, 8610™; Northern Pigments magnetites, NP604™, NP-608™; Magnox magnetites TMB-100™, or TMB-104™; and the like. As colored pigments, there can be selected cyan, magenta, yellow, red, green, brown, blue or mixtures thereof. Generally, cyan, magenta, or yellow pigments or dyes, or mixtures thereof, are used. The pigment or pigments are generally used as water based pigment dispersions.

Specific examples of pigments include SUNSPERSE 6000, FLEXIVERSE and AQUATONE water based pigment dispersions from SUN Chemicals. HELIOGEN BLUE L6900™, D6840™, D7080™, D7020™, PYLAM OIL BLUE™, PYLAM OIL YELLOW™, PIGMENT BLUE 1™ available from Paul Uhlich & Company, Inc., PIGMENT VIOLET 1™, PIGMENT RED 48™, LEMON CHROME YELLOW DCC1026™, E.D. TOLUIDINE RED™ and BON RED C™ available from Dominion Color Corporation, Ltd., Toronto, Ontario, NOVAPERM YELLOW FGL™, HOSTAPERM PINK E™ from Hoechst, and CINQUASIA MAGENTA™ available from E.I. DuPont de Nemours & Company, and the like. Generally, colorants that can be selected are black, cyan, magenta, or yellow, and mixtures thereof. Examples of magentas are 2,9-dimethyl-substituted quinacridone and anthraquinone dye identified in the Color Index as CI-60710, CI Dispersed Red 15, diazo dye identified in the Color Index as CI-26050, CI Solvent Red 19, and the like. Illustrative examples of cyans include copper tetra(oc-tadecyl sulfonamido) phthalocyanine, x-copper phthalocyanine pigment listed in the Color Index as CI-74160, CI Pigment Blue, Pigment Blue 15:3, and Anthrathrene Blue, identified in the Color Index as CI-69810, Special Blue X-2137, and the like. Illustrative examples of yellows are diarylide yellow 3,3-dichlorobenzidene acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33 2,5-dimethoxy-4-sulfonanilide phenylazo-4'-chloro-2,5-dimethoxy acetoacetanilide, and Permanent Yellow FGL. Colored magnetites, such as mixtures of MAPICO BLACK™, and cyan components may also be selected as colorants. Other known colorants can be selected, such as Levanyl Black A-SF (Miles, Bayer) and Sunperse Carbon Black LHD 9303 (Sun Chemicals), and colored dyes such as Neopen Blue (BASF), Sudan Blue OS (BASF), PV Fast Blue B2G01 (American Hoechst), Sunperse Blue BHD 6000 (Sun Chemicals), Irgalite Blue BCA (Ciba-Geigy), Paliogen Blue 6470 (BASF), Sudan III (Matheson, Coleman, Bell), Sudan II (Matheson, Coleman, Bell), Sudan IV (Matheson, Coleman, Bell), Sudan Orange G (Aldrich), Sudan Orange 220 (BASF), Paliogen Orange 3040 (BASF), Ortho Orange OR 2673 (Paul Uhlich), Paliogen Yellow 152, 1560 (BASF), Lithol Fast Yellow 0991K (BASF), Paliotol Yellow 1840 (BASF), Neopen Yellow (BASF), Novoperm Yellow FG 1 (Hoechst), Permanent Yellow YE 0305 (Paul Uhlich), Lumogen Yellow D0790 (BASF), Sunperse Yellow YHD 6001 (Sun Chemicals), Suco-Gelb L1250 (BASF), Suco-Yellow D1355 (BASF), Hostaperm Pink E (American Hoechst), Fanal Pink D4830 (BASF), Cinquasia Magenta

## 12

(DuPont), Lithol Scarlet D3700 (BASF), Toluidine Red (Aldrich), Scarlet for Thermoplast NSD PS PA (Ugine Kuhlmann of Canada), E.D. Toluidine Red (Aldrich), Lithol Rubine Toner (Paul Uhlich), Lithol Scarlet 4440 (BASF), Bon Red C (Dominion Color Company), Royal Brilliant Red RD-8192 (Paul Uhlich), Oracet Pink RF (Ciba-Geigy), Paliogen Red 3871K (BASF), Paliogen Red 3340 (BASF), Lithol Fast Scarlet L4300 (BASF), combinations of the foregoing, and the like.

## 10 Wax

In addition to the polymer binder resin and IR absorber, the toners of the present disclosure also optionally contain a wax, which can be either a single type of wax or a mixture of two or more different waxes. A single wax can be added to toner formulations, for example, to improve particular toner properties, such as toner particle shape, presence and amount of wax on the toner particle surface, charging and/or fusing characteristics, gloss, stripping, offset properties, and the like. Alternatively, a combination of waxes can be added to provide multiple properties to the toner composition.

Optionally, a wax may also be combined with the resin, IR absorber, and optional UV additive in forming toner particles. When included, the wax may be present in an amount of, for example, from about 1 weight percent to about 25 weight percent of the toner particles, in embodiments from about 5 weight percent to about 20 weight percent of the toner particles.

Waxes that may be selected include waxes having, for example, a weight average molecular weight of from about 30 500 to about 20,000, in embodiments from about 1,000 to about 10,000. Waxes that may be used include, for example, polyolefins such as polyethylene, polypropylene, and polybutene waxes such as commercially available from Allied Chemical and Petrolite Corporation, for example POLY-35 WAX™ polyethylene waxes from Baker Petrolite, wax emulsions available from Michaelman, Inc. and the Daniels Products Company, EPOLENE N-15™ commercially available from Eastman Chemical Products, Inc., and VISCOL 55-PTM, a low weight average molecular weight polypropylene available from Sanyo Kasei K. K.; plant-based waxes, such as carnauba wax, rice wax, candelilla wax, sumacs wax, and jojoba oil; animal-based waxes, such as beeswax; mineral-based waxes and petroleum-based waxes, such as montan wax, ozokerite, ceresin, paraffin wax, microcrystalline wax, 40 and Fischer-Tropsch wax; ester waxes obtained from higher fatty acid and higher alcohol, such as stearyl stearate and behenyl behenate; ester waxes obtained from higher fatty acid and monovalent or multivalent lower alcohol, such as butyl stearate, propyl oleate, glyceride monostearate, glyceride distearate, and pentaerythritol tetra behenate; ester waxes obtained from higher fatty acid and multivalent alcohol multimers, such as diethyleneglycol monostearate, dipropylene-glycol distearate, diglyceryl distearate, and triglyceryl tetrastearate; sorbitan higher fatty acid ester waxes, such as 45 sorbitan monostearate, and cholesterol higher fatty acid ester waxes, such as cholesteryl stearate. Examples of functionalized waxes that may be used include, for example, amines, amides, for example AQUA SUPERSLIP6550™, SUPER-SLIP 6530™ available from Micro Powder Inc., fluorinated waxes, for example POLYFLUO 190™, POLYFLUO200™, POLYSILK 19™, POLYSILK 14™ available from Micro Powder Inc., mixed fluorinated, amide waxes, for example MICROSPERSION 19™ also available from Micro Powder Inc., imides, esters, quaternary amines, carboxylic acids or 50 acrylic polymer emulsion, for example JONCRYL 74™, 89™, 130™, 537™, and 538™, all available from SC Johnson Wax, and chlorinated polypropylenes and polyeth-

## 13

ylenes available from Allied Chemical and Petrolite Corporation and SC Johnson wax. Mixtures and combinations of the foregoing waxes may also be used in embodiments. Waxes may be included as, for example, fuser roll release agents.

## Toner Preparation

The toner particles may be prepared by any method within the purview of one skilled in the art. Although embodiments relating to toner particle production are described below with respect to emulsion-aggregation processes, any suitable method of preparing toner particles may be used, including chemical processes, such as suspension and encapsulation processes disclosed in U.S. Pat. Nos. 5,290,654 and 5,302,486, the disclosures of each of which are hereby incorporated by reference in their entirety. In embodiments, toner compositions and toner particles may be prepared by aggregation and coalescence processes in which small-size resin particles are aggregated to the appropriate toner particle size and then coalesced to achieve the final toner-particle shape and morphology.

In embodiments, toner compositions may be prepared by emulsion-aggregation processes, such as a process that includes aggregating a mixture of an optional wax and any other desired or required additives, and emulsions including the resins and IR absorbers described above, optionally in surfactants as described above, and then coalescing the aggregate mixture. A mixture may be prepared by adding an optional wax or other materials, which may also be optionally in a dispersion(s) including a surfactant, to the emulsion, which may be a mixture of two or more emulsions containing the resin and IR absorber. The pH of the resulting mixture may be adjusted by an acid such as, for example, acetic acid, nitric acid or the like. In embodiments, the pH of the mixture may be adjusted to from about 2 to about 4.5. Additionally, in embodiments, the mixture may be homogenized. If the mixture is homogenized, homogenization may be accomplished by mixing at about 600 to about 4,000 revolutions per minute. Homogenization may be accomplished by any suitable means, including, for example, an IKA ULTRA TURRAX T50 probe homogenizer.

Following the preparation of the above mixture, an aggregating agent may be added to the mixture. Any suitable aggregating agent may be utilized to form a toner. Suitable aggregating agents include, for example, aqueous solutions of a divalent cation or a multivalent cation material. The aggregating agent may be, for example, polyaluminum halides such as polyaluminum chloride (PAC), or the corresponding bromide, fluoride, or iodide, polyaluminum silicates such as polyaluminum sulfosilicate (PASS), and water soluble metal salts including aluminum chloride, aluminum nitrite, aluminum sulfate, potassium aluminum sulfate, calcium acetate, calcium chloride, calcium nitrite, calcium oxybate, calcium sulfate, magnesium acetate, magnesium nitrate, magnesium sulfate, zinc acetate, zinc nitrate, zinc sulfate, zinc chloride, zinc bromide, magnesium bromide, copper chloride, copper sulfate, and combinations thereof. In embodiments, the aggregating agent may be added to the mixture at a temperature that is below the glass transition temperature (T<sub>g</sub>) of the resin.

The aggregating agent may be added to the mixture utilized to form a toner in an amount of, for example, from about 0.1% to about 8% by weight, in embodiments from about 0.2% to about 5% by weight, in other embodiments from about 0.5% to about 5% by weight, of the resin in the mixture, although the amounts can be outside of these ranges. This provides a sufficient amount of agent for aggregation.

## 14

The gloss of a toner may be influenced by the amount of retained metal ion, such as Al<sup>3+</sup>, in the particle. The amount of retained metal ion may be further adjusted by the addition of EDTA. In embodiments, the amount of retained crosslinker, for example Al<sup>3+</sup>, in toner particles of the present disclosure may be from about 0.1 pph to about 1 pph, in embodiments from about 0.25 pph to about 0.8 pph, in embodiments about 0.5 pph.

In order to control aggregation and coalescence of the particles, in embodiments the aggregating agent may be metered into the mixture over time. For example, the agent may be metered into the mixture over a period of from about 5 to about 240 minutes, in embodiments from about 30 to about 200 minutes, although more or less time may be used as desired or required. The addition of the agent may also be done while the mixture is maintained under stirred conditions, in embodiments from about 50 rpm to about 1,000 rpm, in other embodiments from about 100 rpm to about 500 rpm, and at a temperature that is below the glass transition temperature of the resin as discussed above, in embodiments from about 30° C. to about 90° C., in embodiments from about 35° C. to about 70° C.

The particles may be permitted to aggregate until a predetermined desired particle size is obtained. A predetermined desired size refers to the desired particle size to be obtained as determined prior to formation, and the particle size being monitored during the growth process until such particle size is reached. Samples may be taken during the growth process and analyzed, for example with a Coulter Counter, for average particle size. The aggregation thus may proceed by maintaining the elevated temperature, or slowly raising the temperature to, for example, from about 40° C. to about 100° C., and holding the mixture at this temperature for a time from about 0.5 hours to about 6 hours, in embodiments from about hour 1 to about 5 hours, while maintaining stirring, to provide the aggregated particles. Once the predetermined desired particle size is reached, then the growth process is halted. In embodiments, the predetermined desired particle size is within the toner particle size ranges mentioned above.

The growth and shaping of the particles following addition of the aggregation agent may be accomplished under any suitable conditions. For example, the growth and shaping may be conducted under conditions in which aggregation occurs separate from coalescence. For separate aggregation and coalescence stages, the aggregation process may be conducted under shearing conditions at an elevated temperature, for example of from about 40° C. to about 90° C., in embodiments from about 45° C. to about 80° C., which may be below the glass transition temperature of the resin as discussed above.

## Shell Resin

In embodiments, an optional shell may be applied to the formed aggregated toner particles. Any resin described above as suitable for the core resin may be utilized as the shell resin. The shell resin may be applied to the aggregated particles by any method within the purview of those skilled in the art. In embodiments, the shell resin may be in an emulsion including any surfactant described above. The aggregated particles described above may be combined with said emulsion so that the resin forms a shell over the formed aggregates. In embodiments, an amorphous polyester may be utilized to form a shell over the aggregates to form toner particles having a core-shell configuration.

The shell resin may be present in an amount of from about 20 percent to about 30 percent by weight of the toner particles, in embodiments from about 24 percent to about 28 percent by weight of the toner particles. In embodiments the IR absorber

as described above may be included in the shell. Thus, the IR absorber may be in the core, the shell, or both.

The IR absorber may thus be present in an amount of from about 0.01 percent to about 5 percent by weight of the toner particles, in embodiments from about 0.5 percent to about 2 percent by weight of the toner particles.

Emulsions of the present disclosure including the resins described above and optional additives may possess particles having a size of from about 100 nm to about 260 nm, in embodiments from about 105 nm to about 185 nm. Toners may have an IR absorber in an amount from about 0.01 percent by weight to about 2 percent by weight of the toner, in embodiments from about 0.10 percent by weight to about 1 percent by weight of the toner, in embodiments from about 0.2 percent by weight to about 0.5 percent by weight of the toner.

Emulsions including these resins may have a solids loading of from about 10% solids by weight to about 25% solids by weight, in embodiments from about 12% solids by weight to about 20% solids by weight, in embodiments about 17% solids by weight.

Once the desired final size of the toner particles is achieved, the pH of the mixture may be adjusted with a base to a value of from about 6 to about 10, and in embodiments from about 6.2 to about 7. The adjustment of the pH may be utilized to freeze, that is to stop, toner growth. The base utilized to stop toner growth may include any suitable base such as, for example, alkali metal hydroxides such as, for example, sodium hydroxide, potassium hydroxide, ammonium hydroxide, combinations thereof, and the like. In embodiments, ethylene diamine tetraacetic acid (EDTA) may be added to help adjust the pH to the desired values noted above. The base may be added in amounts from about 2 to about 25 percent by weight of the mixture, in embodiments from about 4 to about 10 percent by weight of the mixture.

#### Coalescence

Following aggregation to the desired particle size, with the formation of an optional shell as described above, the particles may then be coalesced to the desired final shape, the coalescence being achieved by, for example, heating the mixture to a temperature of from about 55° C. to about 100° C., in embodiments from about 65° C. to about 75° C., in embodiments about 70° C., which may be below the melting point of the crystalline resin to prevent plasticization. Higher or lower temperatures may be used, it being understood that the temperature is a function of the resins used for the binder.

Coalescence may proceed and be accomplished over a period of from about 0.1 to about 9 hours, in embodiments from about 0.5 to about 4 hours, although periods of time outside of these ranges can be used.

After coalescence, the mixture may be cooled to room temperature, such as from about 20° C. to about 25° C. The cooling may be rapid or slow, as desired. A suitable cooling method may include introducing cold water to a jacket around the reactor. After cooling, the toner particles may be optionally washed with water, and then dried. Drying may be accomplished by any suitable method for drying including, for example, freeze-drying.

#### Additives

In embodiments, the toner particles may also contain other optional additives, as desired or required. For example, the toner may include positive or negative charge control agents, for example in an amount of from about 0.1 to about 10 percent by weight of the toner, in embodiments from about 1 to about 3 percent by weight of the toner. Examples of suitable charge control agents include quaternary ammonium compounds inclusive of alkyl pyridinium halides; bisulfates;

alkyl pyridinium compounds, including those disclosed in U.S. Pat. No. 4,298,672, the disclosure of which is hereby incorporated by reference in its entirety; organic sulfate and sulfonate compositions, including those disclosed in U.S. Pat. No. 4,338,390, the disclosure of which is hereby incorporated by reference in its entirety; cetyl pyridinium tetrafluoroborates; distearyl dimethyl ammonium methyl sulfate; aluminum salts such as BONTRON E84™ or E88™ (Hodogaya Chemical); combinations thereof, and the like. Such charge control agents may be applied simultaneously with the shell resin described above or after application of the shell resin.

There can also be blended with the toner particles external additive particles including flow aid additives, which additives may be present on the surface of the toner particles. Examples of these additives include metal oxides such as titanium oxide, silicon oxide, tin oxide, mixtures thereof, and the like; colloidal and amorphous silicas, such as AERO-SIL®, metal salts and metal salts of fatty acids inclusive of zinc stearate, aluminum oxides, cerium oxides, and mixtures thereof. Each of these external additives may be present in an amount of from about 0.1 percent by weight to about 5 percent by weight of the toner, in embodiments of from about 0.25 percent by weight to about 3 percent by weight of the toner, although amounts outside these ranges can be used. Suitable additives include those disclosed in U.S. Pat. Nos. 3,590,000, 3,800,588, and 6,214,507, the disclosures of each of which are hereby incorporated by reference in their entirety. Again, these additives may be applied simultaneously with a shell resin described above or after application of the shell resin.

The characteristics of the toner particles may be determined by any suitable technique and apparatus. Volume average particle diameter  $D_{50v}$ , GSD<sub>v</sub>, and GSD<sub>n</sub> may be measured by means of a measuring instrument such as a Beckman Coulter Multisizer 3, operated in accordance with the manufacturer's instructions. Representative sampling may occur as follows: a small amount of toner sample, about 1 gram, may be obtained and filtered through a 25 micrometer screen, then put in isotonic solution to obtain a concentration of about 10%, with the sample then run in a Beckman Coulter Multisizer 3. Toners produced in accordance with the present disclosure may possess excellent charging characteristics when exposed to extreme relative humidity (RH) conditions. The low-humidity zone (C zone) may be about 10° C./15% RH, while the high humidity zone (A zone) may be about 28° C./85% RH. Toners of the present disclosure may also possess a parent toner charge per mass ratio (Q/M) of from about -3  $\mu$ C/g to about -45  $\mu$ C/g, in embodiments from about -10  $\mu$ C/g to about -40  $\mu$ C/g, and a final toner charging after surface additive blending of from -10  $\mu$ C/g to about -45  $\mu$ C/g.

Utilizing the methods of the present disclosure, desirable gloss levels may be obtained. Thus, for example, the gloss level of a toner of the present disclosure may have a gloss as measured by Gardner Gloss Units (ggu) of from about 20 ggu to about 100 ggu, in embodiments from about 50 ggu to about 95 ggu, in embodiments from about 60 ggu to about 90 ggu.

In embodiments, toners of the present disclosure may be utilized as ultra low melt (ULM) toners. In embodiments, the dry toner particles, exclusive of external surface additives, may have the following characteristics:

(1) Volume average diameter (also referred to as "volume average particle diameter") of from about 2.5 to about 20 microns, in embodiments from about 2.75 to about 10 microns, in other embodiments from about 3 to about 9 microns.

(2) Number Average Geometric Standard Deviation (GSD<sub>n</sub>) and/or Volume Average Geometric Standard Deviation (GSD<sub>v</sub>) of from about 1.05 to about 1.55, in embodiments from about 1.1 to about 1.4.

(3) Circularity of from about 0.9 to about 1 (measured with, for example, a Sysmex FPIA 2100 analyzer), in embodiments from about 0.93 to about 0.99, in other embodiments from about 0.95 to about 0.98.

(4) Glass transition temperature of from about 35° C. to about 60° C., in embodiments from about 37° C. to about 45° C.

(5) The toner particles can have a surface area, as measured by the well known BET method, of about 1.3 to about 6.5 m<sup>2</sup>/g. For example, for cyan, yellow and black toner particles, the BET surface area can be less than 2 m<sup>2</sup>/g, such as from about 1.4 to about 1.8 m<sup>2</sup>/g, and for magenta toner, from about 1.4 to about 6.3 m<sup>2</sup>/g.

It may be desirable in embodiments that the toner particle possess separate crystalline polyester and wax melting points and amorphous polyester glass transition temperature as measured by DSC, and that the melting temperatures and glass transition temperature are not substantially depressed by plasticization of the amorphous or crystalline polyesters, or by the IR absorber, or any optional wax. To achieve non-plasticization, it may be desirable to carry out the emulsion aggregation at a coalescence temperature of less than the melting point of the crystalline component and wax components.

#### Developers

The toner particles thus formed may be formulated into a developer composition. The toner particles may be mixed with carrier particles to achieve a two-component developer composition. The toner concentration in the developer may be from about 1% to about 25% by weight of the total weight of the developer, in embodiments from about 2% to about 15% by weight of the total weight of the developer.

#### Carriers

Examples of carrier particles that can be utilized for mixing with the toner include those particles that are capable of triboelectrically obtaining a charge of opposite polarity to that of the toner particles. Illustrative examples of suitable carrier particles include granular zircon, granular silicon, glass, steel, nickel, ferrites, iron ferrites, silicon dioxide, and the like. Other carriers include those disclosed in U.S. Pat. Nos. 3,847,604, 4,937,166, and 4,935,326.

The selected carrier particles can be used with or without a coating. In embodiments, the carrier particles may include a core with a coating thereover which may be formed from a mixture of polymers that are not in close proximity thereto in the triboelectric series. The coating may include fluoropolymers, such as polyvinylidene fluoride resins, terpolymers of styrene, methyl methacrylate, and/or silanes, such as triethoxy silane, tetrafluoroethylenes, other known coatings and the like. For example, coatings containing polyvinylidene-fluoride, available, for example, as KYNAR 301FTM, and/or polymethylmethacrylate, for example having a weight average molecular weight of about 300,000 to about 350,000, such as commercially available from Soken, may be used. In embodiments, polyvinylidenefluoride and polymethylmethacrylate (PMMA) may be mixed in proportions of from about 30 to about 70 weight % to about 70 to about 30 weight %, in embodiments from about 40 to about 60 weight % to about 60 to about 40 weight %. The coating may have a coating weight of, for example, from about 0.1 to about 5% by weight of the carrier, in embodiments from about 0.5 to about 2% by weight of the carrier.

In embodiments, PMMA may optionally be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, or t butylaminoethyl methacrylate, and the like. The carrier particles may be prepared by mixing the carrier core with polymer in an amount from about 0.05 to about 10 percent by weight, in embodiments from about 0.01 percent to about 3 percent by weight, based on the weight of the coated carrier particles, until adherence thereof to the carrier core by mechanical impaction and/or electrostatic attraction.

Various effective suitable means can be used to apply the polymer to the surface of the carrier core particles, for example, cascade roll mixing, tumbling, milling, shaking, electrostatic powder cloud spraying, fluidized bed, electrostatic disc processing, electrostatic curtain, combinations thereof, and the like. The mixture of carrier core particles and polymer may then be heated to enable the polymer to melt and fuse to the carrier core particles. The coated carrier particles may then be cooled and thereafter classified to a desired particle size.

In embodiments, suitable carriers may include a steel core, for example of from about 25 to about 100 µm in size, in embodiments from about 50 to about 75 µm in size, coated with about 0.5% to about 10% by weight, in embodiments from about 0.7% to about 5% by weight of a conductive polymer mixture including, for example, methylacrylate and carbon black using the process described in U.S. Pat. Nos. 5,236,629 and 5,330,874.

The carrier particles can be mixed with the toner particles in various suitable combinations. The concentrations are may be from about 1% to about 20% by weight of the toner composition. However, different toner and carrier percentages may be used to achieve a developer composition with desired characteristics.

#### Imaging

The toners can be utilized for electrophotographic processes, including those disclosed in U.S. Pat. No. 4,295,990, the disclosure of which is hereby incorporated by reference in its entirety. In embodiments, any known type of image development system may be used in an image developing device, including, for example, magnetic brush development, jumping single-component development, hybrid scavengelss development (HSD), and the like. These and similar development systems are within the purview of those skilled in the art.

Imaging processes include, for example, preparing an image with an electrophotographic device including a charging component, an imaging component, a photoconductive component, a developing component, a transfer component, and a fusing component. In embodiments, the development component may include a developer prepared by mixing a carrier with a toner composition described herein. The electrophotographic device may include a high speed printer, a black and white high speed printer, a color printer, and the like.

Once the image is formed with toners/developers via a suitable image development method such as any one of the aforementioned methods, the image may then be transferred to an image receiving medium such as paper and the like. In embodiments, the toners may be used in developing an image in an image-developing device utilizing a fuser roll member. Fuser roll members are contact fusing devices that are within the purview of those skilled in the art, in which heat and pressure from the roll may be used to fuse the toner to the

image-receiving medium. In embodiments, the fuser member may be heated to a temperature above the fusing temperature of the toner, for example to temperatures of from about 70° C. to about 160° C., in embodiments from about 80° C. to about 150° C., in other embodiments from about 90° C. to about 140° C. (although temperatures outside these ranges can be used), after or during melting onto the image receiving substrate.

In embodiments, the fusing of the toner image can be conducted by any conventional means, such as combined heat and pressure fusing such as by the use of heated pressure rollers. This irradiation step can be conducted, for example, in the same fusing housing and/or step where conventional fusing is conducted, or it can be conducted in a separate irradiation fusing mechanism and/or step. In some embodiments, this irradiation step may provide non-contact fusing of the toner, so that conventional pressure fusing may not be required.

For example, in embodiments, the irradiation can be conducted in the same fusing housing and/or step where conventional fusing is conducted. In embodiments, the irradiation fusing can be conducted substantially simultaneously with conventional fusing, such as by locating an irradiation source immediately before or immediately after a heated pressure roll assembly. Desirably, such irradiation is located immediately after the heated pressure roll assembly, such that crosslinking occurs in the already fused image.

In other embodiments, the irradiation can be conducted in a separate fusing housing and/or step from a conventional fusing housing and/or step. For example, the irradiation fusing can be conducted in a separate housing from the conventional such as heated pressure roll fusing. That is, the conventionally fused image can be transported to another development device, or another component within the same development device, to conduct the irradiation fusing. In this manner, the irradiation fusing can be conducted as an optional step, for example to irradiation cure images that require improved high temperature document offset properties, but not to irradiation cure images that do not require such improved high temperature document offset properties. The conventional fusing step thus provides acceptable fixed image properties for moist applications, while the optional irradiation curing can be conducted for images that may be exposed to more rigorous or higher temperature environments.

In other embodiments, the toner image can be fused by irradiation and optional heat, without conventional pressure fusing. This may be referred to, in embodiments, as noncontact fusing. The irradiation fusing can be conducted by any suitable irradiation device, and under suitable parameters, to cause the desired degree of crosslinking of the unsaturated polymer. Suitable non-contact fusing methods are within the purview of those skilled in the art and include, in embodiments, flash fusing, radiant fusing, and/or steam fusing. These non-contact fusing processes do not require the application of pressure for toner fixation. In embodiments, flash fusing may be utilized. Examples of flash fusing processes which may be utilized include those using xenon lamps, laser fixing processes using a high-intensity laser, combinations thereof, and the like. In embodiments, a non-contact fuser utilized in accordance with the present disclosure may include a source of infrared light operating at a wavelength of from about 750 nm to about 2500 nm.

In embodiments, non-contact fusing may occur by exposing the toner to infrared light at a wavelength of from about 700 to about 850, in embodiments from about 725 to about

845, for a period of time of from about 5 milliseconds to about 2 seconds, in embodiments from about 50 milliseconds to about 1 second.

Where heat is also applied, the image can be fused by irradiation such as by infrared light, in a heated environment such as from about 100 to about 250° C., such as from about 125 to about 225° C. or from about 150 or about 160 to about 180 or about 190° C.

Exemplary apparatuses for producing these images may 10 include, in embodiments, a heating device possessing heating elements, an optional contact fuser, a non-contact fuser such as a radiant fuser, an optional substrate pre-heater, an image bearing member pre-heater, and a transducer. Examples of such apparatus include those disclosed in U.S. Pat. No. 7,141, 15 761, the disclosure of which is hereby incorporated by reference in its entirety.

When the irradiation fusing is applied to the IR absorber-containing toner composition, the resultant fused image is provided with non document offset properties, that is, the 20 image does not exhibit document offset, at temperature up to about 90° C., such as up to about 85° C. or up to about 80° C. The resultant fused image also exhibits improved abrasion resistance and scratch resistance as compared to conventional fused toner images. Such improved abrasion and scratch 25 resistance is beneficial, for example, for use in producing book covers, mailers, and other applications where abrasion and scratches would reduce the visual appearance of the item. Improved resistance to solvents is also provided, which is also 30 beneficial for such uses as mailers, and the like. These properties are particularly helpful, for example, for images that must withstand higher temperature environments, such as automobile manuals that typically are exposed to high temperatures in glove compartments or printed packaging materials that must withstand heat sealing treatments.

It is envisioned that the toners of the present disclosure may 35 be used in any suitable procedure for forming an image with a toner, including in applications other than xerographic applications.

The following Examples are being submitted to illustrate 40 embodiments of the present disclosure. These Examples are intended to be illustrative only and are not intended to limit the scope of the present disclosure. Also, parts and percentages are by weight unless otherwise indicated. As used herein, "room temperature" refers to a temperature of from about 20° C. to about 30° C.

## EXAMPLES

### Example 1

Preparation of Crystalline Resin Emulsion Including a Crystalline Polyester Resin, Copoly(Ethylene-Dodecanoate)-Copoly-(Ethylene-Fumarate), Derived from Dodecanedioic Acid, Ethylene Glycol and Fumaric Acid

55 A one liter Parr reactor equipped with a heating mantle, mechanical stirrer, bottom drain valve and distillation apparatus was charged with dodecanedioic acid (about 443.6 grams), fumaric acid (about 18.6 grams), hydroquinone (about 0.2 grams), n-butylstannoic acid (FASCAT 4100) 60 catalyst (about 0.7 grams), and ethylene glycol (about 248 grams). The materials were stirred and slowly heated to about 150° C. over about 1 hour under a stream of CO<sub>2</sub>. The temperature was then increased by about 15° C. and subsequently about 10° C. intervals, every 30 minutes, to about 180° C.

65 During this time, water was distilled as a by product. The temperature was then increased by about 5° C. intervals over about a 1 hour period to about 195° C. The pressure was then

21

reduced to about 0.03 mbar over about a 2 hour period and any excess glycols were collected in the distillation receiver. The resin was returned to atmospheric pressure under a stream of CO<sub>2</sub> and then trimellitic anhydride (about 12.3 grams) was added. The pressure was slowly reduced to about 0.03 mbar over about 10 minutes and held there for about another 40 minutes. The crystalline resin, copoly(ethylene-dodecanoate)-copolymers-(ethylene-fumarate), was returned to atmospheric pressure and then drained through the bottom drain valve to give a resin with a viscosity of about 87 Pa·s (measured at about 85° C.), an onset melting of about 69° C., melt point temperature peak of about 78° C., and recrystallization peak on cooling of about 56° C. as measured by the Dupont Differential Scanning calorimeter. The acid value of the resin was found to be about 12 meq/KOH.

About 816 grams of ethyl acetate was added to about 125 grams of the above crystalline resin. The resin was dissolved by heating to about 65° C. on a hot plate and stirring at about 200 rpm. In a separate 4 liter glass reactor vessel was added about 4.3 grams of TAYCA POWER surfactant (from Tayca Corporation (Japan), a branched sodium dodecyl benzene sulfonate) (about 47% aqueous solution), about 2.2 grams of sodium bicarbonate (for acid number of approximately 12 meq/KOH) and about 708.33 grams of deionized water was added. This aqueous solution was heated to about 65° C. on a hot plate with stirring at about 200 rpm.

The dissolved resin in ethyl acetate mixture was slowly poured into the 4 liter glass reactor containing the aqueous solution with homogenization at about 4,000 rpm. The homogenizer speed was then increased to 10,000 rpm and left for about 30 minutes. The homogenized mixture was placed in a heat jacketed PYREX distillation apparatus, with stirring at about 200 rpm. The temperature was ramped up to about 80° C. at about 1° C./minute. The ethyl acetate was distilled from the mixture at about 80° C. for about 120 minutes. The mixture was cooled to below about 40° C. then screened through a 20 micron screen. The mixture was pH adjusted to about 7 using about 4% NaOH aqueous solution and centrifuged. The resulting resin included about 35.1% solids by weight in water, with a volume average diameter of about 108 nanometers as measured with a HONEYWELL MICROTAC® UPA150 particle size analyzer.

#### Comparative Example 1

A clear toner, with no IR absorber, was prepared as follows. In a two liter beaker, about 816 grams of ethyl acetate was added to about 125 grams of an amorphous polyester resin, commercially available as XP777 resin, from Reichold Chemicals. The resin was dissolved by heating to about 65° C. on a hot plate and stirring at about 200 rpm. In a separate 4 liter glass reactor vessel, about 3.05 grams (for an acid number of about 17) of sodium bicarbonate was added to about 708.33 grams of deionized water. This aqueous solution was heated to about 65° C. on a hot plate with stirring at about 200 rpm. The dissolved amorphous resin and ethyl acetate mixture was slowly poured into the 4 liter glass reactor containing this aqueous solution with homogenization at about 4,000 rpm. The homogenizer speed was then increased to about 10,000 rpm and left for about 30 minutes. The homogenized mixture was placed in a heat jacketed PYREX distillation apparatus, with stirring at about 200 rpm. The temperature was ramped up to about 80° C. at a rate of about 1° C./minute. The ethyl acetate was distilled from the mixture at about 80° C. for about 120 minutes. The mixture was cooled to below about 40° C. then screened through a 20 micron screen. The mixture was pH adjusted to about 7 using about

22

4% NaOH solution and centrifuged. The resulting resin included about 35.3% solids by weight in water, with particles having a volume average diameter of about 122 nanometers as measured with a HONEYWELL MICROTAC® UPA150 particle size analyzer.

Into a 2 liter glass reactor equipped with an overhead stirrer and heating mantle, about 183.25 grams of the above amorphous resin emulsion and about 104.03 grams of the unsaturated crystalline polyester resin emulsion of Example 1 (about 16.15 weight % crystalline resin) was added. About 41.82 grams of Al<sub>2</sub>(SO<sub>4</sub>)<sub>3</sub> solution (1 weight %) was added as a flocculent under homogenization. The mixture was subsequently heated to about 46.2° C. for aggregation at about 300 rpm. The particle size was monitored with a Coulter Counter until the core particles reached a volume average particle size of 4.59 μM with a GSD of about 1.25, and then about 85.52 grams of the above amorphous resin emulsion was added as a shell, resulting in core-shell structured particles with an average particle size of about 6.48 microns, and a GSD of about 1.23. Thereafter, the pH of the reaction slurry was increased to about 7.2 using about 1.615 grams of ethylene diamine tetraacetic acid (EDTA) about (39 weight %) and NaOH (about 4 weight %) to freeze the toner growth.

After freezing, the reaction mixture was heated to about 69.9° C., and the pH was reduced to about 5.97 for coalescence. The toner was quenched after coalescence, and it had a final particle size of about 5.90 microns, a GSD of about 1.25, and a circularity of about 0.960. The toner slurry was then cooled to room temperature, separated by sieving (through a 25 micron sieve), filtered, washed, and freeze dried.

#### Examples 2 to 4

A toner was prepared with about 0.2 weight percent of IR absorber. An emulsion was first prepared including about 99.8% by weight of an amorphous resin, XP777, available from Reichold Chemicals and 0.2% by weight of an IR absorber as follows. About 125 grams of an amorphous resin XP777 was combined with about 0.24 grams of an IR absorber (either NK-2911 or NK-4680 cyanines (from Hayashibara Biochemical Laboratories, Inc.), or EPO-LIGHT™ 4113, a platinum containing dye (from EPOLIN, Inc.)), and dissolved in a 2 liter beaker containing about 900 grams of ethyl acetate. The mixture was stirred at about 300 revolutions per minute at room temperature to dissolve the resin and IR absorber in the ethyl acetate. About 2.56 grams of sodium bicarbonate was measured into a 3 liter Pyrex glass flask reactor containing about 700 grams of deionized water. Homogenization of the water solution in the 3 liter glass flask reactor was commenced with an IKA Ultra Turrax T50 homogenizer operating at about 4,000 revolutions per minute. The resin solution was slowly poured into the water solution as the mixture continued to be homogenized, and the homogenizer speed was increased to about 8,000 revolutions per minute and homogenization was carried out at these conditions for about 30 minutes. Upon completion of homogenization, the glass flask reactor and its contents were placed in a heating mantle and connected to a distillation device. The mixture was stirred at about 275 revolutions per minute and the temperature of the mixture was increased to about 80° C. at about 1° C. per minute to distill off the ethyl acetate from the mixture.

Stirring of the mixture continued at about 80° C. for about 180 minutes followed by cooling at about 2° C. per minute to room temperature. The product was screened through a 25

micron sieve. The resulting resin emulsion included about 19.61 percent by weight solids in water, with an average of about 135 to 200 nm.

A toner was prepared with the above IR/amorphous resin emulsion as follows. Into a 2 liter glass reactor, equipped with an overhead stirrer and heating mantle, was added about 367.16 grams of the above emulsion containing the amorphous resin and IR absorber. Also added was about 48 grams of an unsaturated crystalline polyester resin of Example 1. About 35.84 grams of  $\text{Al}_2(\text{SO}_4)_3$  solution (about 1 weight %) was added as a flocculent under homogenization. The mixture was subsequently heated to about 40.8° C. for aggregation at about 260 rpm. The particle size was monitored with a Coulter Counter until the core particles reached a volume average particle size of about 4.54  $\mu\text{m}$  with a GSD of about 1.21.

About 171.34 grams of the above amorphous resin and IR absorber emulsion was then added to form a shell, resulting in core-shell structured particles with an average particle size of about 5.77 microns, and a GSD of about 1.22. Thereafter, the pH of the reaction slurry was increased to about 7.25 using about 1.39 grams EDTA (about 39 weight %) and NaOH (about 4 weight %) to freeze the toner growth.

After freezing, the reaction mixture was heated to about 69° C., and the pH was reduced to about 5.9 for coalescence. The toner was quenched after coalescence. The toner slurry

region. FIG. 3 is the UV-Vis-IR spectrum of the amorphous resin co-emulsified with 0.2 wt % of the NK-2911 IR absorber. The mixture was dissolved in ethyl acetate and had a peak at about 836 nm. The peak from about 200 nm to about 320 nm was the absorption of the amorphous resin.

#### Fusing Results

Unfused toner images were made using a Xerox DC12 printer (S/N=FU0-025042) and imaged onto 120 gsm DCEG (Digital Color Elite Gloss, P/N 3R11450) coated paper. A slightly higher than nominal (0.48  $\text{mg}/\text{cm}^2$ ) toner mass area (TMA) was used to obtain a more uniform image quality. The developer charge was 35 grams of toner and 365 grams of Xerox DC-12 carrier. Good quality images were made with the EA toners. The target image used for these test was a solid area patch positioned near the center of the page.

Non-contact fusing was carried out with an IR heater module mounted over a belt transport system. A Heraeus IR emitter was used for this test, short wavelength of 1.2-1.4 microns, with 3 twin tube lamps at 5.4 k Watts. Print samples were carried under the IR lamps at various transport speeds (in mm/seconds (mm/s)) as listed in Table 2 below, as well as the gloss measurements. The color results, showing the difference in color ( $\Delta E 2000$ ) relative to the sample without IR absorber for the test runs, are summarized in Table 3 below.

TABLE 2

| Average Print Gloss at Various Speed |               |             |                                |                                 |                                 |
|--------------------------------------|---------------|-------------|--------------------------------|---------------------------------|---------------------------------|
| Toner                                | Absorber      | Wave length | Speed 88 (mm/s)<br>Gloss (ggu) | Speed 121 (mm/s)<br>Gloss (ggu) | Speed 158 (mm/s)<br>Gloss (ggu) |
| Comparative                          | None          | —           | 52.2 +/- 2.0                   | 13.9 +/- 1.1                    | 7.7 +/- 0.6                     |
| Example 1                            |               |             |                                |                                 |                                 |
| Example 2                            | NK2911        | 831         | 56.8 +/- 0.6                   | 24.4 +/- 3.0                    | 8.3 +/- 0.8                     |
| Example 3                            | NK4680        | 813.5       | 55.5 +/- 2.9                   | 27.8 +/- 4.0                    | 8.5 +/- 2.2                     |
| Example 4                            | EPOLIGHT 4113 | 833         | 58.9 +/- 2.3                   | 24.0 +/- 3.7                    | 10.0 +/- 1.0                    |

TABLE 3

| Color Properties (Delta E 2000) |               |           |                            |                            |                            |
|---------------------------------|---------------|-----------|----------------------------|----------------------------|----------------------------|
| Toner                           | Absorber      | Max. abs. | Speed 120 (mm/s)<br>DE2000 | Speed 120 (mm/s)<br>DE2000 | Speed 154 (mm/s)<br>DE2000 |
| Comparative                     | None          | —         | 0.0                        | 0.8                        | 1.1                        |
| Example 1                       |               |           |                            |                            |                            |
| Example 2                       | NK2911        | 831       | 4.9                        | 4.6                        | 4.7                        |
| Example 3                       | NK4680        | 813.5     | 7.0                        | 6.9                        | 6.9                        |
| Example 4                       | EPOLIGHT 4113 | 833       | 2.0                        | 1.5                        | 1.5                        |

was then cooled to room temperature, separated by sieving (with a 25 micron sieve), filtered, washed, and freeze dried.

A summary of the IR absorbers utilized to produce these toners, as well as the final particle size and circularity obtained, are set forth below in Table 1.

TABLE 1

| Toners including an amorphous resin, crystalline resin, and IR absorber. |               |                      |                     |
|--------------------------------------------------------------------------|---------------|----------------------|---------------------|
| Toner                                                                    | IR absorber   | Toner size (microns) | GSD (volume/number) |
| Comparative                                                              | None          | 5.97                 | 1.25/1.27           |
| Example 1                                                                |               |                      | 0.96                |
| Example 2                                                                | NK-2911       | 5.77                 | 1.24/1.23           |
| Example 3                                                                | NK-4680       | 5.60                 | 1.23/1.23           |
| Example 4                                                                | EPOLIGHT 4113 | 5.54                 | 1.23/1.25           |

UV-Vis-NIR spectra of some of the above components and compositions were obtained utilizing a Cary 5000 Spectrometer from Varian Inc.

FIG. 1 is the UV-Vis-IR spectrum obtained for the NK-2911 IR absorber, which shows that the IR absorber had maximum absorption at about 831 nm when dissolved in MeOH. FIG. 2 is the UV-Vis-IR spectrum of the amorphous resin in THF, showing that it only had absorption in the UV

region. FIG. 3 is the UV-Vis-IR spectrum of the amorphous resin co-emulsified with 0.2 wt % of the NK-2911 IR absorber. The mixture was dissolved in ethyl acetate and had a peak at about 836 nm. The peak from about 200 nm to about 320 nm was the absorption of the amorphous resin.

It will be appreciated that various of the above-disclosed and other features and functions, or alternatives thereof, may be desirably combined into many other different systems or applications. Also that various presently unforeseen or unanticipated alternatives, modifications, variations or improvements therein may be subsequently made by those skilled in the art which are also intended to be encompassed by the following claims. Unless specifically recited in a claim, steps or components of claims should not be implied or imported from the specification or any other claims as to any particular order, number, position, size, shape, angle, color, or material.

What is claimed is:

1. A toner consisting of a core of at least one amorphous resin; an infrared absorber; at least one crystalline resin; a shell of an amorphous resin and an infrared absorber; a colorant; and an optional wax, wherein each infrared absorber has a maximum absorption of light at wavelengths of from about 730 nm to about 800 nm, wherein said infrared absorber is free of absorbance in a wavelength of from about 380 nm to about 700 nm, wherein each infrared absorber is selected from the group consisting of:



and wherein the toner is for use in non-contact fixing.

2. The toner according to claim 1, wherein the toner is an emulsion aggregation toner.

3. The toner according to claim 1, wherein the amorphous resin is an amorphous polyester selected from the group consisting of poly(propoxylated bisphenol co-fumarate), poly(ethoxylated bisphenol co-fumarate), poly(butylxoylated bisphenol co-fumarate), poly(co-propoxylated bisphenol co-ethoxylated bisphenol co-fumarate), poly(1,2-propylene fumarate), poly(propoxylated bisphenol co-maleate), poly(ethoxylated bisphenol co-maleate), poly(butylxoylated bisphenol co-maleate), poly(co-propoxylated bisphenol co-ethoxylated bisphenol co-maleate), poly(1,2-propylene maleate), poly(propoxylated bisphenol co-itaconate), poly(ethoxylated bisphenol co-itaconate), poly(butylxoylated bisphenol co-itaconate), poly(co-propoxylated bisphenol co-ethoxylated bisphenol co-itaconate), poly(1,2-propylene itaconate), and combinations thereof.

4. The toner according to claim 1, wherein the crystalline resin is selected from the group consisting of poly(ethylene-adipate), poly(propylene-adipate), poly(butylene-adipate), poly(pentylene-adipate), poly(hexylene-adipate), poly(octylene-adipate), poly(ethylene-succinate), poly(propylene-succinate), poly(butylene-succinate), poly(pentylene-succinate), poly(hexylene-succinate), poly(hexylene-succinate), poly(octylene-succinate), poly(ethylene-sebacate), poly(propylene-sebacate), poly(butylene-sebacate), poly(pentylene-sebacate), poly(hexylene-sebacate), poly(octylene-sebacate), alkali copoly(5-sulfophthaloyl)-copoly(ethylene-adipate), poly(decylene-sebacate), poly(decylene-decanoate), poly(ethylene-decanoate), poly(ethylene-dodecanoate), poly(nonylene-sebacate), poly(nonylene-decanoate), copoly(ethylene-

fumarate)-copoly(ethylene-sebacate), copoly(ethylene-fumarate)-copoly(ethylene-decanoate), copoly(ethylene-fumarate)-copoly(ethylene-dodecanoate), and combinations thereof.

5. The toner according to claim 1, wherein the colorant consists of dyes, pigments, combinations of dyes, combinations of pigments, or combinations of dyes and pigments in an amount of from about 0.1 to about 35 percent by weight of the toner, and wherein the optional wax is present and is selected from the group consisting of polyolefins, carnauba wax, rice wax, candelilla wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentaerythritol tetra behenate, diethylenglycol monostearate, dipropylene glycol distearate, diglyceryl distearate, triglyceryl tetra stearate, sorbitan monostearate, cholesteryl stearate, and combinations thereof, present in an amount from about 1 weight percent to about 25 weight percent of the toner.

6. The toner according to claim 1, wherein particles comprising the toner are from about 2.75 microns to about 10 microns in diameter, and possess a circularity of from about 0.93 to about 0.99.

7. The toner according to claim 1, wherein the toner possesses a gloss of from about 20 ggu to about 100 ggu, and a parent toner charge per mass ratio of from about -10  $\mu$ C/g to about -40  $\mu$ C/g.

8. A toner consisting of a core containing an amorphous polyester resin; one infrared absorber; a crystalline polyester; a colorant; and a wax wherein the infrared absorber has a maximum absorption of light at wavelengths of from about 730 nm to about 800 nm and does not absorb light at wavelengths of from about 380 nm to about 700 nm, and a shell covering the core, said shell containing an amorphous polyester resin and an infrared absorber, wherein each infrared absorber is selected from the group consisting of:



wherein the toner possesses a gloss of from about 20 ggu to about 100 ggu, and a toner charge per mass ratio of from about -10  $\mu$ C/g to about -40  $\mu$ C/g.

9. The toner according to claim 8, wherein the toner is an emulsion aggregation toner.

10. The toner according to claim 8, wherein the amorphous polyester is of the formula:



wherein m is from about 5 to about 1000.

11. The toner according to claim 8, wherein the crystalline polyester resin is of the formula:



wherein b is from about 5 to about 2000 and d is from about 5 to about 2000.

12. The toner according to claim 8, wherein the colorant consists of dyes, pigments, combinations of dyes, combinations of pigments, or combinations of dyes and pigments in an amount of from about 0.1 to about 35 percent by weight of the toner, and wherein the wax is selected from the group consisting of polyolefins, carnauba wax, rice wax, candelilla wax, sumacs wax, jojoba oil, beeswax, montan wax, ozokerite, ceresin, paraffin wax, microcrystalline wax, Fischer-Tropsch wax, stearyl stearate, behenyl behenate, butyl stearate, propyl oleate, glyceride monostearate, glyceride distearate, pentaerythritol tetra behenate, diethyleneglycol monostearate, dipropylene glycol distearate, diglyceryl distearate, triglyceryl tetra stearate, sorbitan monostearate, cholesteryl stearate, and combinations thereof, present in an amount from about 1 weight percent to about 25 weight percent of the toner.

13. The toner according to claim 8, wherein particles of the toner are from about 2.75 microns to about 10 microns in diameter, and possess a circularity of from about 0.93 to about 0.99.

15 14. A toner consisting of a core containing an amorphous polyester resin; an infrared absorber; a crystalline polyester; a colorant; a shell covering the core said shell containing an amorphous polyester resin and an infrared absorber, wherein the infrared absorber has a maximum absorption of light at wavelengths of from about 730 nm to about 800 nm and does not absorb light at wavelengths of from about 380 nm to about 700 nm, and wherein said infrared absorber present in an amount of from about 0.01 to about 5 percent by weight of toner solids is selected from the group consisting of

25



\* \* \* \* \*